

Patented Aug. 13, 1929.

1,724,522

# UNITED STATES PATENT OFFICE.

MOISEY M. SEREBRIANOI, OF SALTYKOVKA, UNION OF SOCIALIST SOVIET REPUBLICS,  
RUSSIA.

## PAPER MANUFACTURING.

No Drawing. Application filed September 26, 1928, Serial No. 308,572, and in the Union of Soviet  
Republics December 23, 1925.

My invention relates to paper manufacturing and has a particular reference to paper products made of vegetable fibrous waste materials of different kind also to the 5 process of manufacturing paper products from such waste materials.

The object of my invention is to provide a method whereby commercial grades of paper and paper board can be manufactured 10 from cheap waste materials, such as ordinary wood of different grades, bark, sawdust, moss, dried grass, straw, waste paper, rags, cork, etc.

These materials are dried in order to reduce the moisture content to about 4-6% 15 then ground and powdered in suitable machines such as high speed roller mills with blowers, ball mills, stone grinding mills, etc. The powdered material is screened and the 20 tailings are powdered again. Ordinary air separators may be used for this purpose, also shakers and rotary screens of a type used in flour and cement mills.

The powdered material is placed in a tank 25 with an agitator and a mixture of equal quantities of turpentine and gasoline (or benzin), or turpentine and kerosene, are added, a total of from 6 to 10% by weight.

In order to obtain a more uniform mixture 30 it is recommended to use an excess of the above mixture of gasoline and turpentine (or similar hydrocarbons). A portion of this mixture can be recovered when mixing operation is completed, by squeezing or 35 pressing out from the pulp, or by some other method.

If it is desired to produce a very soft and flexible paper then rubber should be added to the pulp, about 2-4% by weight, or a corresponding amount of powdered leather 40 scrap.

After the pulp has been thoroughly mixed 45 with added hydrocarbons it is used for making paper or paper board by one of the following methods:

1. The paper and board are made by a process similar to the one used in rubber manufacture, i. e. by drawing the pulp between hot and cold rolls until the desired 50 thickness and density are obtained.

2. The prepared mass or pulp is fed into the pit of an ordinary paper machine provided with a suitable agitator, which is nec-

essary for a continuous and thorough mixing. The process of making paper is then 55 continued as with an ordinary paper pulp.

The paper and paper board obtained by my method possess all the properties of ordinary commercial products of this kind, being considerably cheaper for the manufacture, 60 as I am using cheap waste materials for same. The properties of the finished product may be varied according to requirements by modifying the composition as it was explained above. 65

I claim as my invention:

1. In a process of manufacturing paper, consisting in grinding and pulverizing a mixture of dried vegetable waste materials, mixing said materials with turpentine, and 70 drawing the resultant mixture into sheets.

2. In a process of manufacturing paper, consisting in grinding and pulverizing a mixture of dried vegetable waste materials, mixing said materials with turpentine and 75 with mineral hydrocarbon, and drawing the resultant mixture into sheets.

3. In a process of manufacturing paper, consisting in grinding and pulverizing dried wood, bark, sawdust, grass, straw, paper, 80 rags, cork, or the like, mixing said matter with turpentine and mineral hydrocarbon, and drawing the resultant mixture into sheets.

4. In a process of manufacturing paper, 85 consisting in grinding and pulverizing wood, bark, sawdust, grass, straw, paper, rags, cork, leather, or the like, mixing said materials with turpentine and mineral hydrocarbons, adding rubber, and drawing the resultant mixture into sheets. 90

5. In a process of manufacturing paper, consisting in grinding and pulverizing dried wood, bark, sawdust, grass, straw, paper, 95 rags, cork, or the like, adding from 6 to 10 percent of a mixture of equal parts of turpentine and a mineral hydrocarbon, and drawing the resultant mixture into sheets.

6. In a process of manufacturing paper, consisting in grinding and pulverizing dried 100 fibrous materials, adding from 6 to 10 percent of a mixture of turpentine with mineral hydrocarbon, and drawing the resultant mixture into sheets.

7. In a composition matter for manufacturing paper, consisting of a mixture of 105

finely ground fibrous materials with turpen-  
tine and mineral hydrocarbon.

8. In a composition matter for manufac-  
turing paper, consisting of a mixture of fine-  
ly ground dried fibrous materials with tur-  
pentine and mineral hydrocarbon.

9. In a composition matter for manufac-  
turing paper, consisting of a mixture of fine-  
ly ground dried fibrous materials with a  
10 mixture of turpentine and mineral hydro-  
carbon, said last named substances being  
taken in approximately equal proportions.

10. In a paper, made of finely ground  
dried fibrous materials mixed with turpen-  
tine and mineral hydrocarbon.

11. A paper, made of finely ground dried  
fibrous materials mixed with from 6 to 10  
percent of a mixture of turpentine and a  
mineral hydrocarbon.

Signed at the city of Riga, Republic of 20  
Latvia, this twentieth day of August A. D.  
1928.

MOISEY M. SEREBRIANOI.